

## UNITED STATES PATENT OFFICE

2,403,104

## LITHIUM GREASES

Elvin B. Lien, Berkeley, Calif., assignor to Union  
Oil Company of California, Los Angeles, Calif.,  
a corporation of California

No Drawing. Application October 17, 1942,  
Serial No. 462,413

13 Claims. (Cl. 252—42)

1

This invention relates to lubricating greases, and the principal object thereof is to produce a stable lubricating grease free from tendency to "bleed" and to increased starting and running torque at low temperatures, and which is at the same time both water-resistant and stable to temperature fluctuations and pressure changes.

Primarily, the invention resides in a lithium soap grease which is rendered particularly suitable for extremely low temperature use, wherein the low temperature properties are imparted through the presence of a small proportion, e. g. 5%, of a so-called unsaponifiable oil obtained as a by-product from the production of soaps from acidic materials produced by oxidation of highly paraffinic petroleum lubricating oil. Also, the lithium soap grease produced under this invention is rendered particularly stable against leakage of oil or tendency to "bleed" or "weep." Furthermore, such products are found to be appreciably improved in physical appearance in that they are unusually clear and brilliant in comparison with greases not containing the unsaponifiable oil.

The lithium soap used in the grease may be prepared in any known or preferred manner from any appropriate fatty acid or other soap-making acidic material suitable for grease manufacture. For example, a suitable grease may be made from lithium stearate which is produced in any appropriate manner from commercial stearic acid, such as by reacting lithium carbonate or other suitable lithium base with stearic acid. Similarly, other fatty acids such as oleic acid, palmitic acid and the like or mixtures of these acids may be used according to well understood soap-making procedure. Thus, both animal and vegetable fatty acid may be employed.

These lithium soaps may be employed in suitable mineral lubricating oils in varying proportions according to the particular type of grease desired. Normally, the stiffer the grease desired, the greater the soap proportions. Whereas, a thin grease might contain only 1% or 2% of the soap, heavier-bodied greases will contain from 4% or 5% of soap up to 10% or 15% or any other desired proportion. Such greases have been described in patents issued to Clarence E. Earle Nos. 2,274,673, 2,274,674, 2,274,675 and 2,274,676, and various acidic materials appropriate therefor are indicated in those patents. In addition it may be desirable for some uses to use other acidic materials such as naphthenic acids derived from petroleum whereby lithium naphthenates are produced. It may also be desirable for some pur-

5 poses to employ synthetic acids produced by oxidation of lubricating oils, or the sulfonic acids obtained as a by-product in the manufacture of white oils.

10 The present improvement renders greases of this type thoroughly stable, especially for low temperature uses such as for airplane lubrication, and protects them against a tendency to leak or "bleed" some of the oil, especially where it is important to use low viscosity lubricating oils. This tendency is controlled or completely overcome by the employment therein of a small percentage, such as 5%, of the indicated unsaponifiable oil or oily material which is recovered in connection with the production of metal soaps from the oxidation products of the modern highly paraffinic lubricating oils such as those which are produced by solvent extraction of paraffin base oils.

15 20 In connection with the production of some types of lubricants, various so-called highly paraffinic lubricating oil fractions, such as just indicated, are subjected to oxidation, as by air blowing, to produce acidic materials. This oxidation may take place under elevated temperatures and pressures, such as the temperatures between about 280° F. and 350° F. and under pressures between about 50 lbs. and 200 lbs. A typical operation is to air-blow at a temperature of about 320° F. and 25 under a pressure of 95 lbs. gage. Air blowing is carried on for a time to produce commercially maximum oxidation or other substantial degree of oxidation. The oxidation batch which then contains substantial amounts of acidic materials, 30 as indicated by a typical saponification value of 80, is then reacted with sodium hydroxide, or other suitable base at a temperature of 250° F. and a pressure of 60 lbs. per square inch, to form the desired sodium soap or other desired metal salt. Separation of the unsaponifiable oil is realized by mixing the sodium soap and oil with a quantity of water, e. g. 25% water, heating the batch to around 180° F. to 200° F., agitating, and allowing the whole to settle. The soap layer settles to the bottom leaving an emulsion layer in the middle and a relatively clear unsaponifiable oil on top. The soap and emulsion layers are easily separated from the unsaponified oils which consist principally of unoxidized hydrocarbons, 35 ketones, esters and the like and possibly a small proportion of dissolved soap.

40 45 50 55 It is the above described unoxidized by-product oil which is meant by the term "unsaponifiable oil from petroleum oxidation processes," or similar term, as herein used.

It has been discovered that when minor proportions of this oil are used in the lubricating oil employed in the grease production, an otherwise present tendency of the grease to bleed out some of the oil is overcome. This function is especially desirable where low viscosity oils, such as transformer oils or very light lubricating oils are employed for the grease production. In addition to reducing this sweating tendency, the described unsaponifiable oil also imparts appreciable physical difference in that the product containing the unsaponifiable oil is clearer and almost transparent, as distinguished from a grease without it which is usually opaque or at best only translucent. Perhaps this difference in appearance is due to the effect of the unsaponifiable oil in rendering the soap more compatible with the oil. Of even more importance than the reduction in bleeding and improvement in physical appearance of greases produced with unsaponifiable oil are the lower operating temperatures to which the grease can be subjected without appreciably increasing its starting or running torque.

The amount of saponifiable oil may vary from the indicated 5%. For example, as little as about 2% is effective in lowering torque, reducing bleeding of oil, and rendering the product clearer. Again, larger proportions such as 6% or 8% may be introduced with increase in the desirable effects, up to an unsaponifiable oil content of about 10%, beyond which there does not appear to be a constantly increasing appreciable improvement. However, at least for some uses, it is possible to replace all of the lubricating oil in the grease with said unsaponifiable oil, providing the viscosity is appropriate. Thus, lubricating oils from a grade of about SAE 10 up to a grade of about SAE 40 may be oxidized, and the unsaponifiable oils recovered after saponification of the oxidation batches having respectively viscosities corresponding with SAE grades from about 10 to 70.

With respect to lubricating oils to be employed in preparing the grease, these may be selected according to ordinary grease practices. Thus, the oil may be of naphthenic type or paraffinic type, or of mixed base, as desired, and obviously, the viscosity of the oil will vary with the grease required.

In connection with avoidance of torque increase at low temperatures tests were made with a test shaft rotating in a packed bearing and under a constant force, using greases made with transformer oil, as in the following table:

| Grease | Composition     |                  |                    | Temp. | Seconds for one rotation |
|--------|-----------------|------------------|--------------------|-------|--------------------------|
|        | Transformer oil | Lithium stearate | Unsaponifiable oil |       |                          |
| A      | Percent         | Percent          | Percent            | ° F.  |                          |
| A      | 94.3            | 5.7              | None               | -67   | 1,300                    |
| B      | 89.3            | 5.7              | 5.0                | -67   | 430                      |
| C      | 91.0            | 9.0              | None               | -55   | 1,000                    |
| D      | 86.0            | 9.0              | 5.0                | -55   | 120                      |

This shows a reduction in torque to about one-third where substituting 5% unsaponifiable oil in same A to produce sample B and a reduction to about one-eighth where making a similar substitution in sample C (where the soap content is greater) to produce sample D.

In addition to employing the described unsaponifiable oil for the purposes indicated, it is sometimes desirable to add an oxidation inhibitor,

inasmuch as there is sometimes a tendency for lithium greases to darken substantially after manufacture. A very desirable material for this purpose has been found to be phenyl alpha naphthylamine. An adequate proportion is about 0.2% of the grease, but this may be varied according to the extent of control desired from perhaps as little as 0.05% to perhaps as much as 1.0%, although greater proportions than 1.0% can be employed, if desired, to further increase the oxidation resistance of the grease. Another suitable anti-oxidant is p-phenylene diamine. Also, other high boiling point arylamines and other inhibitors may be employed in somewhat similar proportions.

In addition to employing lithium soaps, such as lithium stearate, there are occasional instances where it seems desirable to add smaller proportions of other soaps. For example, about 1/2% to 2% of calcium stearate, sodium stearate, magnesium stearate, or especially aluminum stearate, or soap of similar acid, may be added to a grease containing in the order of 10% of lithium stearate. Similarly, small proportions of these additional soaps may be added to greases containing either less or more lithium stearate, such as to greases containing 4% or 5% of lithium stearate or other lithium soap. The purpose of these additions, when desirable to employ them, is to improve compatibility.

Variations in the product and in the method of its production will be apparent to those skilled in the art. For example, the compatibility-improving soaps may be prepared from any acid previously mentioned for lithium soaps.

I claim:

1. A lubricating grease comprising mineral oil, a minor proportion of lithium soap, and a minor proportion of unsaponifiable oil obtained from the recovery of synthetic acids produced by the oxidation of lubricating oil fractions.
2. A lubricant comprising mineral lubricating oil, about 1% of lithium soap, and a minor proportion of unsaponifiable oil obtained as a by-product after recovery of synthetic acids produced by the oxidation of a petroleum lubricating oil fraction.
3. A lubricant comprising a petroleum fraction of lubricating viscosity, a minor proportion of lithium soap to thicken the oil, and a minor proportion of unsaponifiable oil remaining after recovery of synthetic acids produced by oxidation of a mineral lubricating fraction, the unsaponifiable oil being present in proportion sufficient to reduce tendency to increase torque at sub-normal temperatures.
4. A lubricant according to claim 3 wherein the unsaponifiable oil is present in excess of about 2% of the total composition.
5. A lubricant according to claim 3 wherein the soap is present in proportion in excess of about 1% and the unsaponifiable oil is present in excess of about 2%.
6. A lubricating grease comprising a mineral oil fraction having lubricating viscosity, a minor proportion of lithium soap to thicken the oil, and a minor proportion sufficient to prevent bleeding of unsaponifiable oil obtained after separation of synthetic acids produced by the oxidation of a refined petroleum fraction.
7. A lubricant comprising a petroleum fraction of lubricating viscosity, a minor proportion between about 1% and 25% of lithium soap, and a minor proportion between about 2% and 10% of unsaponifiable oil obtained after separation of

synthetic acids produced by the oxidation of refined petroleum fractions.

8. A lubricant according to claim 7 containing an oxidation inhibitor.

9. A lubricant according to claim 7 containing an oxidation inhibitor of the class consisting of phenyl alpha naphthylamine and p-phenylene diamine.

10. A lubricant according to claim 3 containing phenyl alpha naphthylamine in a minor proportion sufficient to act as an oxidation inhibitor.

11. A lubricant according to claim 3 contain-

ing a minor proportion sufficient to act as a compatibility agent of a soap of the class consisting of calcium, sodium, magnesium and aluminum soaps.

12. A lubricant according to claim 3 containing a high boiling point aryl amine in minor proportion sufficient to act as an oxidation inhibitor.

13. A lubricant according to claim 2 wherein the unsaponifiable oil is present in proportion sufficient to reduce tendency to increased torque at subnormal temperatures.

ELVIN B. LIEN.